

Patented Sept. 13, 1927.

1,642,159

# UNITED STATES PATENT OFFICE.

CHARLES F. KUMLI, OF CHICAGO, ILLINOIS, ASSIGNOR TO SPIEGEL, MAY, STERN COMPANY, OF CHICAGO, ILLINOIS, A CORPORATION OF ILLINOIS.

## STENCIL SHEET.

No Drawing.

Application filed June 14, 1926. Serial No. 116,038.

This invention relates to stencils and particularly to stencil sheets comprising a fibrous, porous support, such as Japanese Yoshino paper, having a hardened coating of organic colloid, impervious to ink, in which the stencil characters are cut to permit the ink or other coloring to print through the fibers of the paper, or other porous support.

10 Heretofore, the impervious film, with which the stencils have been coated, consisted largely of gelatine, which has been objectionable mainly because of its comparatively high price.

15 In order to adapt the coated sheet for making the stencil by pressure, as for instance by the impact of the types of a typewriter, the sheet must be dampened so as to permit the type to rupture the impervious film without cutting or otherwise injuring the fiber of the paper, or other porous support. In dampening coated sheets which have been hardened by aluminum salts alone, the fibers of the paper have a tendency to stretch so as to cause the stencil to become baggy in the frame, and the paper has a tendency to become sticky.

The main objects of this invention are to provide a coating solution for stencil sheets having glue as its principal ingredient to take the place of the more costly gelatine heretofore used; to provide an improved hardening solution for treating the sheets after the impervious film has been applied; 25 to provide a stencil sheet which will not become baggy or sticky after being dampened preparatory to the cutting of the characters; to provide a stencil sheet which is tough and inexpensive, and to provide an improved process of making a stencil sheet of this kind.

30 Stencils may be made of any suitable fibrous material, but Japanese Yoshino paper is preferred because of its thin texture.

In carrying out this invention, the sheet is coated with a solution which preferably includes glue, glycerine, a volatile vehicle, and zinc chloride.

35 The glue is the principal ingredient and gives the sheet the desired ink-resisting surface. A good grade of hide glue has been found to be satisfactory and is much cheaper than the gelatine heretofore used.

The glycerine is a tempering agent. The 55 stencil sheet, after being coated with the solution, is kept in a flexible condition by the glycerine which retains enough moisture to keep the sheet from becoming brittle.

The volatile vehicle may be water or any other suitable solvent which evaporates quickly after the film has been applied to the sheet.

Japanese Yoshino paper tears very easily 65 when moistened and, therefore, there has been considerable waste heretofore in handling the sheets during the coating process. By the addition of zinc chloride to this solution, the fibers of the paper are toughened 70 and tearing of the paper is greatly reduced.

The ingredients of the above solution may be combined in varied proportions, but it has been found that the best results can be obtained from a combination in the following proportions:

|               | Parts<br>by weight. |
|---------------|---------------------|
| Glue          | 22                  |
| Glycerine     | 22                  |
| Water         | 210 80              |
| Zinc chloride | 3                   |

After the sheets are coated with the above solution, they are dried by any suitable means and then coated with a hardening 85 solution including aluminum chloride, glycerine, potassium dichromate and a volatile vehicle.

The aluminum chloride and potassium dichromate are both hardening agents and by 90 using them combined in the hardening solution it has been found that better results are obtained than by using them separately. When stencil sheets are hardened with aluminum salts without the dichromate, the 95 fibers have a tendency to stretch after being moistened, thus causing the sheet to become baggy in the frame. The paper also has a tendency to become sticky. A baggy sheet is very objectionable because of the difficulty 100 in properly aligning the stencil characters during the cutting operation.

When potassium dichromate is used alone as the hardening agent, the sheet must be exposed to light, because the coagulating action of potassium dichromate on the organic colloid is dependent upon a light reaction which consumes considerable time. In or-

der to expose the sheets, so that their entire surface is acted upon by the light, a large amount of floor space is required if the stencils are to be manufactured in considerable quantities. The use of potassium dichromate alone is, therefore, objectionable.

By using the aluminum chloride and potassium dichromate in combination for the hardening solution, the sheets will not be 10 come baggy, when subsequently moistened, and the sheets need not be exposed to the light for a longer period than is required to evaporate the volatile solvent, usually about one hour.

15 Water may be used as the carrying agent in the hardening solution. Glycerine is also used in the hardening solution in order to compensate for any glycerine in the coating solution which may have been dissolved by 20 the water.

The ingredients in the hardening solution may be combined in varied proportions, but it has been found that the best results can be obtained from the following combination:

|                                    | Parts<br>by weight. |
|------------------------------------|---------------------|
| Water                              | 200                 |
| Aluminum chloride                  | 5                   |
| Glycerine                          | 45                  |
| Potassium dichromate solution (6%) | 10                  |

30 The sheet may be coated on either one or both sides in any suitable manner, as by dipping, spraying or by means of a brush, rollers or the like.

35 Although this invention is here particularly described in its preferred embodiment, it will be understood that the product and the various steps of the process may be modified by omission or alteration of details and 40 substitution of ingredients, without departing from the spirit of the invention as defined by the following claims.

I claim:

45 1. A stencil blank comprising a sheet of fibrous material coated with glue and zinc chloride.

2. A stencil blank comprising a sheet of

fibrous material coated with a solution including glue, glycerine and zinc chloride.

3. A stencil blank comprising a sheet of 50 fibrous material coated with a solution including an animal colloid and zinc chloride.

4. A stencil blank comprising, a sheet of fibrous material coated with a solution including glue, glycerine, zinc chloride, and a 55 volatile carrying agent.

5. A stencil blank comprising a sheet of fibrous material coated with a solution including an animal colloid about 22 parts, glycerine about 22 parts, a volatile vehicle 60 about 210 parts, and zinc chloride about 3 parts.

6. A stencil blank comprising a sheet of fibrous material coated with a solution including glue about 22 parts, glycerine about 65 22 parts, water about 210 parts, and zinc chloride about 3 parts.

7. The process of preparing a stencil sheet which consists in coating the sheet with a film including glue, permitting the film to 70 dry, and then coating the film with a hardening solution, including aluminum chloride, glycerine, potassium dichromate and water.

8. A stencil blank comprising a sheet of fibrous material coated with glue, zinc chlo- 75 ride, and potassium dichromate.

9. A stencil blank comprising a sheet of fibrous material coated with a solution including glue, glycerine, zinc chloride and 80 potassium dichromate.

10. A stencil blank comprising a sheet of fibrous material coated with a solution including glue, glycerine, zinc chloride, potassium dichromate and a volatile carrying 85 agent.

11. A stencil blank comprising a sheet of fibrous material coated with a solution including glue, glycerine, zinc chloride, potassium dichromate, aluminum chloride, and 90 a volatile carrying agent.

Signed at Chicago this 5th day of June, 1926.

CHARLES F. KUMLI.